

**1**

3,843,423

**METHOD FOR PRODUCING STEEL SHEETS OR STRIPS FOR MAKING CANS**

Hidejiro Asano, Kitakyushu, and Yashichi Oyagi, Yachiyo-machi, Japan, assignors to Nippon Steel Corporation, Tokyo, Japan

No Drawing. Filed Aug. 23, 1973, Ser. No. 391,020

Claims priority, application Japan, Aug. 24, 1972,

47/84,100

Int. Cl. C21d 9/46

U.S. Cl. 148—12

1 Claim

**ABSTRACT OF THE DISCLOSURE**

A method for producing can-making steel sheet comprising subjecting a steel slab containing not more than 0.03% C, not more than 1.0% Mn, not more than 0.04% P, not more than 0.02% O, with the balance being iron and unavoidable impurities to finish hot rolling at a temperature between the  $A_3$  transformation point and 750° C., coiling the sheet at a temperature not lower than 620° C., and cold rolling thus obtained hot rolled sheet or strip after acid pickling with a reduction rate not lower than 80%.

The present invention relates to a very economical method for producing steel sheets for can-making.

More particularly, the present invention is to provide an economical method for producing steel sheets or strips (herein after called sheets) for can-making, having satisfactory workability (can-making properties) similar or better than those of the can-making steel sheet (so-called twice cold rolled sheet abridged as 2 C R steel sheet) obtained by cold rolling annealed cold rolled sheet again and by metal coating the sheet, or those of the can-making steel sheet obtained by stress-relief annealing a cold rolled steel sheet.

As widely known, very extensive studies have been made for a method for producing low-cost can-making steel sheets in the steel making industry and various proposals have been made up to now. The problem which is most concerned at the present time is to provide steel sheets having satisfactory can-making properties at low cost, and already at the present time some methods have been known for producing relatively low cost can-making steel sheets.

For example, "Progress on Metal Containers," K. W. Brighton, Canned Foods, page 3 and a Japanese Patent Publication Sho 38-8563 disclose a method for producing can-making steel sheets by two-step cold rolling, and Japanese patent publications Sho 41-18486 and Sho 43-12504 disclose a method for producing can-making steel sheets by annealing the sheet at a low temperature for incomplete recrystallization after cold rolling.

However, according to the two-step cold rolling methods disclosed in the above first two prior publications, it is necessary to conduct the first-step cold rolling and annealing and in addition the second-step cold rolling, and according to the methods disclosed in the latter two prior publications, the sheet after the cold rolling is annealed at a low temperature. Although the products produced by the above conventional methods have high strength and good can-making properties, it is necessary in the former method to conduct the additional cold rolling, thus causing disadvantages in respect of equipments and necessity of use of high cost rolling oil as well as provision of a subsequent degreasing line, and the latter method, although advantageous over the former method, has disadvantages in respect of the annealing time and production cost due to the low temperature annealing of cold rolled steel sheets.

**2**

The conventional two-step method for producing can-making steel sheets includes steps of hot rolling—acid pickling—cold rolling—electrolytic degreasing—annealing—second cold rolling—electrolytic degreasing—plating, while the low temperature annealing method includes steps of hot rolling—acid pickling—cold rolling—electrolytic degreasing—stress-relief annealing—shape correcting (may be omitted)—planting. According to the conventional methods, complete annealing is conducted at a temperature higher than 600° C. in order to remove the work hardening effect of the cold rolled steel sheets or stress-relief annealing is conducted at a temperature between 400 and 600° C.

It is clear that if such annealing steps can be omitted, very economical production of can-making steel sheet is possible.

The present invention is based on the above facts and has been completed as a result of extensive studies for obtaining good can-making properties by combination of steel composition and operational conditions of production steps without an annealing step.

The gist of the present invention lies in the method for producing can-making steel sheets which is characterized in that a steel slab containing not more than 0.03% C, not more than 1.0% Mn, not more than 0.04% P, not more than 0.02% O with the balance being iron and unavoidable impurities is subjected to finishing rolling in a temperature range from its  $A_3$  transformation point to 750° C., coiled at a temperature not lower than 620° C., and thus obtained hot rolled steel sheet is acid pickled and cold rolled with a reduction rate not lower than 80%.

More particularly, steel ingot or slab containing not more than 0.03% C, not more than 1.0% Mn, not more than 0.04% P, not more than 0.02% O with the balance being iron and unavoidable impurities is prepared by the conventional mold casting method or continuous casting method, and the slab which produced above method is heated to 1000 to 1300° C. in slab reheating furnace and hot rolled.

In the hot rolling, the temperature when the sheet passes the final rolling rolls, namely the finishing outlet temperature and the coiling temperature are important. According to the present invention, the temperature at the hot rolling finishing outlet should be between the  $A_3$  transformation point of the steel and 750° C. and the coiling temperature should be not less than 620° C. for the reasons herein set forth.

The hot rolled coil thus obtained is acid pickled and cold rolled at a reduction rate not less than 80% into cold rolled strip of 0.1 to 0.5 mm. thickness. This cold rolled strip is directly used as can-making cold rolled steel sheet, and no subsequent annealing for the purpose of stress relief is required.

The reasons for the above limitations in the present invention will be explained hereinunder.

The carbon content is limited to not more than 0.03% for the following reason. It has been conventionally considered that when work strain remains in steel sheet, corrosion resistance is deteriorated, but it has been found by the present inventors that corrosion resistance is remarkably improved by lowering the carbon content to not more than 0.03%, preferably 0.018%, and that some carbon content is necessary for obtaining strength required by cans. Manganese is added to prevent lowering of hot workability of hot rolled sheet due to sulfur and to give the sheet required strength. However, the manganese content should be not more than 1.0%, but in an amount more than three times of the sulfur content. Phosphorus should be not more than 0.04% because it remarkably deteriorates corrosion resistance of the steel sheet. Oxygen is a harmful element, because it combines with manganese

and silicon in the steel to form oxides, thus lowering cleanliness of the steel and deteriorating can-making properties. Particularly high degree of cleanliness of the steel is required when cold rolling of more than 80% reduction rate is done as in the present invention. Thus, the oxygen content is limited to not more than 0.02%. Among the hot rolling conditions, the finishing rolling temperature and the coiling temperature are important for obtaining excellent strength and workability for can-making, particularly in case of cold rolled steel sheets which have been subjected to strong cold reduction. The reason for defining the finishing rolling temperature as between the  $A_3$  transformation point and 750° C. is that this temperature range is optimum for formation of complete equiaxed grains free from hot rolled structure, and the reason for defining the coiling temperature as not lower than 620° C. that this temperature range is desirable for obtaining optimum strength of the sheet for can-making and is desirable from the point of economy.

The advantage of the present invention is that satisfactory workability of the sheet for can-making can be obtained only by the strong cold rolling of more than 80% reduction rate through the combination of the steel composition and the production conditions, and that satisfactory mechanical properties for maintaining require can-strength can be obtained.

Can-making properties of can-making steel sheets produced by the conventional methods as described hereinbefore from steel of the ladle analysis shown in Table 1 are good.

TABLE 1

| C         | Percent of— |           |           |             |           |             |
|-----------|-------------|-----------|-----------|-------------|-----------|-------------|
|           | Si          | Mn        | P         | S           | Cu        | N           |
| 0.04-0.15 | <0.08       | 0.20-0.70 | 0.01-0.14 | 0.015-0.050 | 0.02-0.20 | 0.001-0.025 |

However, the can-making steel stocks produced by the conventional methods require annealing and workability of the sheet as cold rolled with heavy reduction is poor and it is impossible to work the sheet into cans directly.

According to the present invention, excellent can-making properties can be given to the cold rolled steel sheet obtained by strong cold rolling of more than 80% reduction rate thanks to the steel composition as specified above, and no annealing is required after the cold rolling due to the lowered carbon and oxygen contents. In this point, the present invention is essentially different from

of the hot rolling does not exceed the  $A_3$  transformation point of the steel and the sheet is coiled at a temperature not lower than 620° C. The coiled steel strip is maintained at the temperature for substantial time so that the steel is subjected to recrystallization annealing by its own heat and the hot rolled structure is eliminated. When the soft hot rolled steel sheet thus produced is subjected to cold rolling of more than 80% reduction according to the present invention, tensile strength of the sheet as cold rolled will be lower than about 70 kg./mm.<sup>2</sup>, and it is possible to improve the productivity of cans without sacrifice of can-making properties.

For the actual practice of the present invention, steel containing not more than 0.03% C, not more than 1.0% Mn, not more than 0.04% P, not more than 0.02% O with the balance being iron and unavoidable impurities is prepared in an ordinary steel making furnace such as a converter, an open hearth, and an electric furnace. Vacuum degassing may be used to adjust the carbon and oxygen contents.

Thus prepared molten steel is made into slabs by continuous casting or an ordinary ingot-making and breaking-down method and subjected to the steps of hot rolling—acid pickling—cold rolling—degreasing—shape correcting (may be omitted)—plating to obtain the final product. In the plating step, tin-plating, chromium-plating or chemical conversion treatment is effected.

The present invention will be more clearly understood from the following examples.

## EXAMPLE 1

Steel having the composition shown in Table 2 was prepared in a converter and part of the molten steel was subjected to vacuum degassing to adjust the composition. These steels were hot rolled with the finishing outlet temperature at a temperature not higher than the  $A_3$  transformation point, namely between 780 and 840° C. (aiming at 810° C.), and were coiled at 640° C. Thus obtained hot rolled sheets were cold rolled with a reduction rate of 89% into cold rolled steel sheets of 0.26 mm. thickness.

| Number | C     | Si    | Mn   | P     | S     | Cu   | Al    | O     | N      |
|--------|-------|-------|------|-------|-------|------|-------|-------|--------|
| 1      | 0.08  | 0.011 | 0.36 | 0.017 | 0.016 | 0.03 | tr.   | 0.042 | 0.0026 |
| 2      | 0.032 | 0.024 | 0.49 | 0.016 | 0.012 | 0.03 | 0.051 | 0.008 | 0.0059 |
| 3      | 0.007 | 0.023 | 0.28 | 0.010 | 0.021 | 0.05 | 0.004 | 0.035 | 0.0061 |
| 4      | 0.008 | 0.010 | 0.25 | 0.060 | 0.012 | 0.04 | 0.038 | 0.014 | 0.0038 |
| 5      | 0.011 | 0.081 | 0.41 | 0.008 | 0.010 | 0.02 | 0.010 | 0.007 | 0.0041 |
| 6      | 0.008 | 0.021 | 0.33 | 0.014 | 0.024 | 0.03 | 0.072 | 0.006 | 0.0040 |
| 7      | 0.016 | 0.008 | 0.27 | 0.010 | 0.019 | 0.13 | 0.042 | 0.010 | 0.0051 |
| 8      | 0.010 | 0.019 | 0.48 | 0.026 | 0.014 | 0.02 | 0.031 | 0.009 | 0.0068 |

NOTE.—No. 1 to No. 4 are outside the steel composition of the present invention. No. 5 to No. 8 are within the steel composition of the present invention.

Table 3 shows the mechanical properties and workability into beer can lids as well as can-making feasibility of the cold rolled steel sheets thus obtained.

TABLE 3

| Number | Hardness (HR30T) | Tensile strength (kg./mm. <sup>2</sup> ) | Can-making  |             |
|--------|------------------|------------------------------------------|-------------|-------------|
|        |                  |                                          | Workability | Feasibility |
| 1      | 81               | 80                                       | X           |             |
| 2      | 80               | 76                                       | O           | X           |
| 3      | 78               | 68                                       | X           |             |
| 4      | 80               | 78                                       | O           | X           |
| 5      | 77               | 70                                       | O           | O           |
| 6      | 78               | 65                                       | O           | O           |
| 7      | 78               | 69                                       | O           | O           |
| 8      | 77               | 67                                       | O           | O           |

NOTE: (1) Can-making workability is shown by the workability into beer can lids; (2) Can-making feasibility was determined by occurrence of poor seaming in the seaming step after the beer can lid stamping step; (3) No. 1-No. 4 are cold rolled sheets from the steels of No. 1 to No. 4 in Table 2, and No. 5 to No. 8 are cold rolled sheets from the steels of No. 5 to No. 8 in Table 2; (4) O=good, X=bad.

the conventional methods for producing can-making steel sheets. On the other hand, if the steel composition of the present invention is subjected to the finishing outlet temperature of higher than the  $A_3$  transformation point as in the conventional methods, only can-making steel sheet of excessively high strength is obtained, although enough can-making properties are obtained. Such excessively high strength of the can-making steel sheet necessarily causes difficulties in respect of rigidity of the can-making machine and the driving source, and is not always desirable even when satisfactory can-making properties can be obtained. Rather, can-making steel sheets having lower strength as cold rolled condition are increasingly demanded in more and more cases in recent years. In order to obtain tensile strength of not more than about 70 kg./mm.<sup>2</sup> as cold rolled with more than 80% reduction rate, it is necessary that the finishing outlet temperature

No. 1 to No. 4 which are outside the composition of the present invention (No. 1 is outside the composition in respect of C and O, No. 2 in respect of C, No. 3 in respect of O, and No. 4 in respect of P) could not be worked into cans or had poor can-making feasibility even when they had some workability. On the other hand, No. 4 to No. 8, which are within the composition of the present invention, were excellent both in can-making workability and can-making feasibility.

## EXAMPLE 2

Steel having the composition shown in Table 4 was hot rolled under the conditions shown in Table 4 and cold rolled with reduction rate of 87% into cold rolled sheets of 0.27 mm. thickness, and their mechanical properties, workability, can-making feasibility are shown in Table 5. "A" in Table 5 indicates the finishing outlet temperature not lower than the  $A_3$  transformation point, and "B" represents the finishing outlet temperature not higher than the  $A_3$  transformation point. As clearly seen from the results shown in the table, the can-making feasibility of No. 3B which is within the composition of the present invention is poor due to the too low coiling temperature in spite of the finishing rolling temperature below the  $A_3$  transformation point. No. 4, due to its high carbon content, shows slightly lower can-making feasibility in spite of satisfactory hot rolling conditions. On the other hand, No. 1B and No. 2B which are within the scope of the present invention show remarkably excellent can-making feasibility in particular.

TABLE 5

| 5  | Sample No. | Hardness (HR30T) | Tensile strength (kg./mm. <sup>2</sup> ) | Can-making workability | Can-making feasibility |
|----|------------|------------------|------------------------------------------|------------------------|------------------------|
| 10 | (A)        | 81               | 87                                       | O                      | X                      |
|    | (B)        | 78               | 69                                       | O                      | O                      |
| 2  | (A)        | 80               | 82                                       | O                      | X                      |
|    | (B)        | 77               | 65                                       | O                      | O                      |
| 3  | (A)        | 80               | 84                                       | O                      | X                      |
|    | (B)        | 79               | 78                                       | O                      | X                      |
| 4  | (A)        | 82               | 90                                       | O                      | X                      |
|    | (B)        | 79               | 73                                       | O                      | △                      |

NOTE: O=good; △=slightly good; X=bad.

15

What is claimed:

1. A method for producing can-making steel sheet comprising subjecting a steel slab containing not more than 0.03% C, not more than 1.0% Mn, not more than 0.04% P, not more than 0.02% O, with the balance being iron and unavoidable impurities to finish hot rolling at a temperature between the  $A_3$  transformation point and 750° C., cooling the sheet at a temperature not lower than 620° C., and cold rolling thus obtained hot rolled sheet or strip after acid pickling with a reduction rate not lower than 80%.

TABLE 4

| Sample No. | Compositions (percent) |    |       |       |      |       |       |      | Hot rolling condition |                         |                      |
|------------|------------------------|----|-------|-------|------|-------|-------|------|-----------------------|-------------------------|----------------------|
|            | C                      | Si | Mn    | P     | S    | Cu    | Al    | O    | N                     | Finish-ing temp. (° C.) | Coiling temp. (° C.) |
| 1          | {A}                    |    | 0.015 | 0.021 | 0.34 | 0.009 | 0.016 | 0.03 | 0.001                 | 0.009                   | 0.0041               |
|            | {B}                    |    |       |       |      |       |       |      |                       | 905                     | 650                  |
| 2          | {A}                    |    | 0.007 | 0.011 | 0.29 | 0.014 | 0.008 | 0.02 | 0.063                 | 0.007                   | 0.0062               |
|            | {B}                    |    |       |       |      |       |       |      |                       | 800                     | 670                  |
| 3          | {A}                    |    | 0.011 | 0.024 | 0.46 | 0.011 | 0.014 | 0.02 | 0.045                 | 0.012                   | 0.0045               |
|            | {B}                    |    |       |       |      |       |       |      |                       | 920                     | 600                  |
| 4          | {A}                    |    | 0.035 | 0.021 | 0.38 | 0.018 | 0.011 | 0.03 | 0.031                 | 0.010                   | 0.0039               |
|            | {B}                    |    |       |       |      |       |       |      |                       | 820                     | 850                  |

## References Cited

## UNITED STATES PATENTS

- 2,814,578 11/1957 White ----- 148—12  
 3,264,144 8/1966 Frazier et al. ----- 148—12  
 3,614,886 10/1971 Nishihara ----- 148—12

WAYLAND W. STALLARD, Primary Examiner